

# UNITED STATES PATENT OFFICE.

LESTER J. MALONE, OF ROCHESTER, NEW YORK, ASSIGNOR TO EASTMAN KODAK COMPANY, OF ROCHESTER, NEW YORK, A CORPORATION OF NEW YORK.

## PROCESS OF MAKING COLORED NITROCELLULOSE COMPOSITIONS.

1,399,357.

Specification of Letters Patent.

Patented Dec. 6, 1921.

No Drawing.

Application filed April 20, 1921. Serial No. 463,092.

To all whom it may concern:

Be it known that I, LESTER J. MALONE, a citizen of the United States of America, residing at Rochester, in the county of Monroe 5 and State of New York, have invented certain new and useful Improvements in Processes of Making Colored Nitrocellulose Compositions, of which the following is a full, clear, and exact specification.

10 This invention relates to a process of making colored nitrocellulose compositions which can be advantageously used in the plastic arts, such, for instance, as film manufacture and varnish making.

15 One object of my invention is to provide a method of making colored compositions which will yield particularly uniform products. Another object of my invention is to provide a process in which relatively inexpensive and easily manipulated water-soluble dyes may be employed. Other objects 20 will hereinafter appear.

After nitrocellulose is taken from the nitrating acid, substantially all of the latter 25 is removed by careful washing. Such washed nitrocellulose fibers are the preferred material with which my process starts. I immerse or otherwise treat them in an aqueous solution of dye, preferably an acid 30 dye, until they have assumed the proper tint. The strength of the dye bath may be greatly varied, as will be understood by those skilled in this art. The dye solution penetrates very completely throughout all the fibers and the 35 latter are, therefore, dyed with a high degree of uniformity.

When the fibers have taken up the desired amount of color, they are separated from the dye solution, the excess of the latter being 40 washed out.

The colored nitrocellulose fibers are then dehydrated in the manner customary in this art, such as by treatment with butyl alcohol or fusel oil, and are then dissolved up into 45 compositions or dopes. These colored fibers enter properly into all of the usual nitrocellulose compositions, particularly those employed in film manufacture or varnish making. By way of example, but without 50 being in any way limited thereto, it is noted that these fibers can be used in the compositions described in United States Patents Nos. 1,342,602, Seel, June 8, 1920, and 1,370,922, Seel, Combs and Kemp, Mar. 8, 55 1921.

The color or dye passes into the composition or solution along with the fibers and, because of its uniform distribution throughout all the fibers, it gives a uniform color to the dope with the minimum amount of 60 mixing.

I find that the uniformity of dyeing the fibers, which in turn aids in the uniform coloring of the dope, is enhanced by the ability of the aqueous solution of the dye to 65 penetrate very rapidly and easily along the wet washed nitrocellulose fibers.

Where it is desired that the finished compositions have a predetermined depth of color, I have found that my method is particularly useful. By immersing the fibers for a given time in a dye bath of given strength and temperature a definite tint results.

Having thus described my invention, 75 what I claim as new and desire to secure by Letters Patent is:

1. The process of making a colored nitrocellulose composition, which comprises the steps of dying the nitrocellulose fibers and 80 then dissolving said dyed fibers in a nitrocellulose solvent.

2. The process of making a colored nitrocellulose composition, which comprises the steps of coloring nitrocellulose fibers with an 85 aqueous dye bath, removing the surplus dye bath and then dissolving said colored fibers in a nitrocellulose solvent.

3. The process of making colored nitrocellulose compositions, which comprises the 90 steps of treating wet nitrocellulose fibers with an aqueous dye bath until the fibers are colored, then washing away the excess of dye bath from the fibers, dehydrating said fibers and then dissolving the same in a 95 nitrocellulose solvent.

4. The process of making a colored nitrocellulose composition, which comprises the steps of treating washed nitrocellulose fibers with an acid water-soluble dye bath until 100 said fibers are colored, removing the surplus dye bath, dehydrating said fibers, and finally dissolving the same in a nitrocellulose solvent.

Signed at Rochester, New York, this 11th 105 day of April 1921.

LESTER J. MALONE.